

C. PACK,

METHOD OF FORMING DIE CASTINGS.  
APPLICATION FILED JUNE 6, 1918.

1,299,769.

Patented Apr. 8, 1919.

2 SHEETS—SHEET 1.

Fig. 1.



Fig. 2.



Fig. 3.



INVENTOR

Charles Pack  
BY  
J. Edmunds  
ATTORNEY

C. PACK.  
METHOD OF FORMING DIE CASTINGS.  
APPLICATION FILED JUNE 6, 1918.

1,299,769.

Patented Apr. 8, 1919.

2 SHEETS—SHEET 2.



INVENTOR

Charles Pack  
BY  
J. Edmonds  
ATTORNEY

# UNITED STATES PATENT OFFICE.

CHARLES PACK, OF BROOKLYN, NEW YORK, ASSIGNOR TO DOEHLER DIE CASTING COMPANY, OF BROOKLYN, NEW YORK, A CORPORATION OF NEW YORK.

## METHOD OF FORMING DIE-CASTINGS.

1,299,769.

Specification of Letters Patent.

Patented Apr. 8, 1919.

Application filed June 6, 1918. Serial No. 238,481.

*To all whom it may concern:*

Be it known that I, CHARLES PACK, a citizen of the United States, residing in the borough of Brooklyn, county of Kings, and State of New York, have invented certain new and useful Improvements in Methods of Forming Die-Castings, of which the following is a specification.

My invention relates to a method of forming die castings whereby the formation of cracks in the same because of shrinkage stresses will be obviated, and to the castings made by such method as new articles of manufacture. When a sheet or wall of metal is cast between metal dies and the end portions of the same, or portions at some distance from each other are held during the process of casting, so as to prevent shrinkage of the part, considerable stresses will be set up in the metal. Thus, for example, if the wall or partition being considered is one of the sides of a box-like structure or has other walls or parts extending therefrom at an angle, these offset portions being firmly held between the die members of the mold during the solidification and cooling of the casting, it will be obvious that the wall or part will be held against movement in the mold between such offset portions. The metals used for making die castings all have a shrinkage which may be computed as a constant factor per inch of length upon the transition of the metal from the molten to the solid state, and a further shrinkage, the amount of which per inch may readily be figured, during the cooling from the temperature at which the metal solidifies to that at which the casting is removed from the mold. In the case of a wall or part having considerable extent and comparatively thin section, the stresses thus set up when the part is held from decreasing in length in the mold are considerable, and these stresses cause a pull at a point in the wall or part which for some reason may be a weak point, sufficient in many cases to cause a crack at such point. It is evident that the pull at such point will be of an amount equal to the pull per unit length multiplied by the length through which the stress is permitted to act, and the case of a wall having smooth surfaces and held at its ends, the pull or stress at a given distance from an end will be equal to the stress per

unit length multiplied by the distances from the ends or fixed points.

I have found that I can remedy this situation by providing the part which is to be protected against shrinkage with spaced projections on one or both faces of the wall, which projections may be very slight in height, such, for example, as slight ribs formed on the face of the wall at right angles to the direction of the stress. Such projections form points of anchorage between the casting and the adjacent die member, so that the shrinkage stresses in the member will be sub-divided in accordance with the number and spacing of such projections. Thus, for example, if a wall be six inches in length and held at its ends, and if twelve equally spaced ribs are provided between the ends of the wall, the shrinkage stress between any adjacent pair of projections, or between the end wall of the casting and the adjacent projection will be only one-twelfth of the total shrinkage stress developed within the part or wall, all of which stress would exert a pull at one weak point in the wall if the surfaces of the same were smooth. I am, of course, aware of the fact that ribs or projections are often formed on die castings for stiffening purposes or for the purpose of performing some other function in relation to the use for which the casting is intended. My invention does not include the use of such projections, but, on the contrary, relates to the production of slight projections on surfaces which would otherwise be smooth, and which projections are intended to serve no useful end other than to distribute and sub-divide the shrinkage stresses in the part.

In order that a clearer understanding of my invention may be had, attention is hereby directed to the accompanying drawings forming part of this application and illustrating certain embodiments of my invention. In the drawings, Figure 1 represents a top plan view of a casting formed in accordance with my invention, Fig. 2 is a longitudinal section thereof taken on line 2—2 of Fig. 1, Fig. 3 is a transverse section taken on the line 3—3 of Fig. 2, the casting being shown as still within the die in which it is formed, Fig. 4 is a top plan view partly shown in horizontal section of another form of casting embodying my invention, and

Figs. 5 and 6 are sections taken respectively on lines 5—5 and 6—6 of Fig. 4.

Referring to the drawings, the casting 1 shown in Figs. 1, 2 and 3 embodies a construction in which a thin bottom portion 2 is bounded by end walls 3, 3, by a vertical side wall 4 and by a curved side wall 5, having apertured lugs or offset portions 6, 6 at the bottom thereof. The inner surface of the bottom portion 2 would normally be entirely smooth, and because of its large extent relative to its cross section, considerable shrinkage stresses develop therein during the solidification and cooling of the casting. I have shown this bottom portion 2 as protected against such shrinkage stresses by forming thereon a plurality of spaced longitudinal ribs 7, 7 of slight height and a plurality of spaced transverse ribs 8, 8, which may extend between the ribs 7, 7 to form a sort of lattice work, as shown. The casting is shown in Fig. 3 as still within the parts 9, 9' of the die from which is evident the manner in which the bottom wall 2 is restrained from shrinking lengthwise between the end walls 3, 3 and also the manner in which the ribs 7, 7 anchor the bottom portion 2 to the die member 9' and thereby sub-divide the stresses in bottom member 2 between the walls 3, 3. In Figs. 4, 5 and 6 a rectangular frame member 10 is shown, the four sides of which are provided with vertical web portions 11, 11 and with top flange portions 12, 12. The web portions are provided at various points with vertical ribs 13, which are of considerable size, and are provided for the purpose of stiffening the casting or for serving some other purpose in connection with the use for which the casting is intended. In accordance with my invention, I provide the vertical ribs 14, 14 on the inner surfaces of the webs 11 regardless of whether or not the stiffening offsets or lugs 13 are or are not used. The ribs or projections 14 are of slight height and width, are formed on surfaces which would otherwise be smooth and have no purpose other than to sub-divide the shrinkage stresses in the manner indi-

cated. Ribs 14, or other projections for the same purpose, are provided at suitably spaced intervals, which may be calculated with regard to the shrinkage coefficients of the metal of the casting, the distance between offset portions of the walls of the casting and the other physical factors of the problem.

What I claim is:—

1. In the method of forming die castings, which comprises forming between rigid dies a metal casting having a wall of considerable extent in proportion to its thickness, with offset portions at the extremities thereof, the step of sub-dividing shrinkage stresses in different sections along the length of the wall between said offset portions, by so forming one of the dies as to provide slight spaced projections on one of the faces of said wall, which projections have no function in relation to the useful purpose of the casting formed, but are provided on a surface which would otherwise be smooth.

2. In the method of forming die castings, which comprises forming between rigid dies a metal casting having a wall of considerable extent in proportion to its thickness, with offset portions at the extremities thereof, the step of providing ribs of slight height on one of the faces of said wall, at spaced intervals between said offset portions, transversely to the direction of the shrinkage stresses between said offset portions, by so forming one of the dies as to form said ribs on said wall, and thereby sub-dividing the stresses tending to crack said wall between said offset portions, when the casting solidifies in the mold and cools, said ribs being formed on a surface which would otherwise be smooth, being unnecessary for stiffening purposes, and having no relation to the useful purpose of the casting formed.

This specification signed and witnessed this 3rd day of June, 1918.

CHARLES PACK.

Witnesses:

EDMUND J. WARD,  
GEO. L. MOORE.